# EUROPEAN PATENT SPECIFICATION

(11) **EP 1 458 899 B1**
(45) Date of publication and mention of the grant of the patent: **21.01.2009**
(21) Application number: 02797006.0
(22) Date of filing: 25.12.2002
(51) Int. Cl.: C23C 2/12

(54) **METHOD OF APPLYING THE COATINGS FROM ALUMINIUM ALLOY ON CAST IRON AND STEEL PRODUCTS**
VERFAHREN ZUM AUFBRINGEN VON ÜBERZÜGEN AUS ALUMINIUMLEGIERUNG AUF GUSSEISEN- UND STAHLPRODUKTE
PROCEDE D'APPLICATION DE REVETEMENTS A BASE D'ALLIAGE D'ALUMINIUM SUR DES PRODUITS EN FONTE ET EN ACIER

(30) Priority: 26.12.2001 RU 2001135068
(43) Date of publication of application: 22.09.2004
(73) Proprietor: Legal and Consulting Agency "JUREPROMCONSULTING" Ltd, Moscow 119607 (RU); Marutian, Sergey Vasilievich, Moscos, 113519 (RU); Volkov, Yuriy Sergeevich, Moscow, 117419 (RU)
(72) Inventor: MARUTIAN, Sergey Vasilievich, Moscow, 113519 (RU); VOLKOV, Yuriy Sergeevich, Moscow, 117419 (RU)
(74) Representative: Laitinen, Pauli Sakari
(86) International application number: PCT/RU2002/000555
(87) International publication number: WO 2003/060180

(56) References cited:
- EP-A- 0 870 847
- EP-A1- 0 545 049
- DE-A1- 2 601 067
- GB-A- 451 771
- GB-A- 975 063
- GB-A- 1 440 328
- RU-C1- 2 059 010
- RU-C1- 2 061 085
- SU-A1- 1 555 374
- SHLUGERA M.A.: 'Spravochnik', vol. 1, 1985, MASHINOSTROENIE, MOSCOW article 'Galvanicheskie pokrytiya v mashinostroenii', pages 63 - 65, XP008097754

## Description

### Technical field

The invention refers to applying metal, e.g. aluminum, coatings by plunging into the melt and may be used, for instance, for corrosion protection of rolled and other cast iron and steel products.

### Background of the invention

Methods of applying the aluminum coatings on steel products by plunging into the aluminum melt comprising zinc and magnesium are known.

The closest analog of the present invention is the method of applying the aluminum coatings on cast iron and steel products comprising product surface preparation and consequent plunging the product into the aluminum melt alloyed with zinc and silicon (GB, Nº 1440328, MPK C23 C1/00,1976).

The disadvantage of the closest analog is impossibility of aluminum melt applying on cast iron and steel products at the temperature lower than 715 C without using fluxes and the presence of intermetallic compounds of quite a big thickness (10-15 micrometers) make the coating brittle, which doesn't allow to deform the steel product with aluminum coating hereinafter. EP-A-870847 disclose a aluminum plating bath comprising silicon set at 660°C for coating steel sheets.
GB-A-975063 disclose a method of coating steel pieces by submerging in a molten aluminum alloy comprising silicon, zinc and magnesium at a temperature of 600 to 800°C. DE-A-2601067 disclose a method of coating iron pieces by blasting and then by dipping in a molten aluminum bath at a temperature of 550 to 950°C.

### Summary of the invention

The present invention solves the problem of decreasing the temperature of aluminum melt, at this temperature the formation of quite a plastic protective coating without using the flux is provided, which allows to deform rolled and other products with aluminum coatings.

In the method of applying the aluminum coatings on cast iron and steel products comprising product surface preparing and consequent plunging the product into the aluminum melt alloyed with zinc and silicon the solution of said problem is reached by jet-abrasive preparing of the product and the aluminum melt is alloyed with zinc, silicon, magnesium, tin of following mass percentage:

| | |
|---|---|
| zinc | 7.0-10.0 |
| silicon | 3.0-5.0 |
| magnesium | 0.5-1.5 |
| tin | 0.2-0.5 |

while the temperature of the melt is in the range of 660 - 680 C.

The results of applying the aluminum coatings, using jet-abrasive preparing of the surface, in melts of different chemical composition, studying the structure and working qualities of the coatings are presented in Table 1.

Plasticity of the coatings was estimated by testing the pattern on bending around the cylindrical mandrel, while wending on which the coating on the pattern doesn't break. Corrosion qualities of the coatings were estimated according to the results of fast tests of patterns treaded with moisture phase film comprising Cl-ion (imitation of the sea atmosphere).

Electrochemical studies of the resulting coating have shown that alloying the aluminum melt, comprising zinc, silicon, magnesium and tin leads to significant increasing in reproducibility of results of electrode potential measurement of the coating, which indicate high uniformity of chemical composition of coating surface layers.

Aluminum coatings were applied on patterns after the jet-abrasive preparing of their surface under different temperature and time regimes by plunging into the melt of the following chemical composition: aluminum - base, zinc - 8.0%, silicon - 4.5%, magnesium - 1.1%, tin - 0.4%. The results of the studies if said coatings are presented in Table 2.

The studies have shown that in temperature range of 660-680 C the formation of thickness uniform aluminum coating without flux using is taking place, this coating is characterized by high corrosion resistance and plasticity.

Analysis of the results of aluminizing in melts of different chemical composition and of different regimes (Tables 1,2) has shown that aluminizing of steel patterns with jet-abrasive preparing of surface in the melt comprising aluminum - base, zinc - 7.0 - 10.0%, silicon - 3.0 -5.0%, magnesium - 0.5 -1.5%, tin - 0.2 - 0.5% at the temperature of 660-680 C leads to the solution of the above said problem. Aluminizing in the proposed melt without flux using and by said regimes provides formation of thickness and structure uniform plastic coatings of high corrosion resistance.

**Table 1.**

| **The main characteristics of aluminum coatings formed in melts of different chemical composition.** | | | | | | |
|---|---|---|---|---|---|---|
| Melt composition | Temperature of applying, C | Time of exposure in the melt, sec | Coating thickness, micrometer | Transition zone thickness, micrometer | Minimum diameter of mandrel, mm | Character of the corrosion |
| Aluminum - base Silicon - 2.0% Manganese - 0.5% | 720 - 740 | 40 | 70 | 50 | - | Pit |
| Aluminum - base Silicon - 7.0% Manganese - 0.5% | 730-750 | 70 | 40 | 20 | 20 | Pit |
| Aluminum - base Zinc - 5.0% Silicon - 2.0% | 690-710 | 60 | 50 | 25 | 15 | General, local |
| Aluminum - base Zinc - 7.0% Silicon- 5.0% | 680-700 | 60 | 70 | 20 | 10 | General, local |
| Aluminum - base Zinc - 10% Silicon- 5.0% | 670-690 | 70 | 60 | 20 | 10 | General, local |
| Aluminum - base Zinc- 10% Silicon- 5.0% Magnesium - 1.0% | 660 -680 | 70 | 70 | 10 | 10 | General |
| Aluminum - base Zinc- 10% Silicon- 5.0% Magnesium - 1.0% Tin- 0.5% | 660 -680 | 70 | 70 | 5 | 10 | General |

**Table 2.**

| **The main characteristics of aluminum coatings formed in the melt of proposed chemical composition.** | | | | | | |
|---|---|---|---|---|---|---|
| Melt composition | Temperature of applying, C | Time of exposure in the melt, sec | Coating thickness, micrometer | Transition zone thickness, micrometer | Minimum diameter of mandrel, mm | Character of the corrosion |
| Aluminum - base | 650 | 120 | 80 | 10 | 15 | General |
| Zinc- 8.0% | 660 | 80 | 70 | 5 | 10 | General |
| Silicon- 4.5% | 670 | 70 | 60 | 5 | 10 | General |
| Magnesium- 1.1% | 680 | 70 | 60 | 5 | 10 | General |
| Tin - 0.4% | 690 | 70 | 70 | 10 | 20 | Local |
| | 700 | 70 | 70 | 15 | 25 | Local |
| | 710 | 80 | 90 | 20 | 30 | Local |

## Claims

1. Method of applying the aluminum coatings on cast iron and steel products comprising product surface preparing and consequent plunging the product into the aluminum melt alloyed with zinc and silicon **characterized by** jet-abrasive preparing of the product and the aluminum melt is alloyed with zinc, silicon, magnesium, tin of following mass percentage:
| | |
|---|---|
| zinc | 7.0-10.0 |
| silicon | 3.0-5.0 |
| magnesium | 0.5-1.5 |
| tin | 0.2-0.5, |
while the temperature of the melt is in the range of 660 - 680 C.

## Patentansprüche

1. Verfahren zur Auftragung von Aluminiumbeschichtungen auf Gusseisen- und Stahlprodukten, bestehend aus Oberflächenvorbehandlung des Produkts und anschließendem Eintauchen des Produkts in die Aluminiumschmelze, die mit Zink und Silizium legiert ist, **gekennzeichnet durch** Wasserstrahl-Vorbehandlung des Produkts und dass die Aluminiumschmelze mit Zink, Silizium, Magnesium, Zinn mit folgenden Massen-Prozentsätzen legiert ist:
Zink 7,0-10,0
Silizium 3,0-5,0
Magnesium 0,5-1,5
Zinn 0,2-0,5,
während die Temperatur der Schmelze in einem Bereich von 660 bis 680° C liegt.

## Revendications

1. Procédé pour l'application de revêtements d'aluminium sur fer moulé et des produits d'acier comprenant la préparation de la surface du produit et ensuite la plongée du produit dans un alliage d'aluminium fondu contenant du zinc et du silicium, **caractérisé par** la préparation du produit au jet abrasif et par l'aluminium fondu est allié avec du zinc, du silicium, du magnésium, de l'étain dans les pourcentages suivants en masse:
| | |
|---|---|
| zinc | 7,0-10,0 |
| silicium | 3,0-5,0 |
| magnésium | 0,5- 1,5 |
| étain | 0,2 - 0,5, |
la température du métal liquide étant dans la gamme de 660 à 680 C.
